

# United States Patent

[11] 3,548,135

[72] Inventor Allan John Wood  
Stafford, England  
[21] Appl. No. 641,880  
[22] Filed May 29, 1967  
[45] Patented Dec. 15, 1970  
[73] Assignee The English Electric Company Limited  
London, England  
a British company  
[32] Priority May 27, 1966  
[33] Great Britain  
[31] No. 23781/66

2,975,256 3/1961 Lee et al. .... 200/166(C)X  
3,042,474 7/1962 Aurand et al. .... 75/173  
3,239,635 3/1966 Baude .... 200/144(.2)  
3,367,801 2/1968 Kreiselmaier .... 75/173X  
FOREIGN PATENTS  
693,827 9/1964 Canada .... 200/144.2

Primary Examiner—Robert S. Macon  
Attorney—Misegades and Douglas

[54] **CONTACTS FOR VACUUM INTERRUPTERS**  
9 Claims, 1 Drawing Fig.

[52] U.S. Cl. .... 200/144,  
200/166, 75/133  
[51] Int. Cl. .... H01h 33/66  
[50] Field of Search. .... 200/144.2,  
166(C); 75/173

[56] **References Cited**

UNITED STATES PATENTS

1,769,229 7/1930 Mandell .... 200/144(.2)  
2,719,085 9/1955 Schatz .... 75/173

**ABSTRACT:** Contacts for vacuum interrupters have their faces, between which an arc may be struck in operation, formed of dissimilar materials, which materials, on arcing between the faces, become intermixed and form nonductile films. The materials are mechanically strong and have high electrical and thermal conductivities.

Preferably the face of one contact is formed of silver-silicon and that of the other is formed of silver-nickel, these materials on arcing forming nonductile layers of nickel silicides on the faces, which markedly reduces the tendency of the contacts to weld together.

In an alternative, the face of one contact may be formed of high-purity zone-refined copper and that of the other of high-purity vacuum outgassed titanium. In this case nonductile films of copper-titanium compounds are formed.



PATENTED DEC 15 1970

3,548,135



INVENTOR  
Allan John Wood  
BY  
Misegades &  
Douglas  
ATTORNEYS

## CONTACTS FOR VACUUM INTERRUPTERS

This invention relates to contacts for vacuum interrupters.

According to this invention a pair of cooperating contacts in or for a vacuum circuit interrupter has parts defining their respective cooperating faces, between which an arc is struck in operation, formed of dissimilar materials, each of which materials is mechanically strong and has high electrical and thermal conductivity, and which materials, on arcing between said cooperating faces, become intermixed and form nonductile films.

Two embodiments of the invention will now be described by way of example, with reference to the accompanying drawing, which shows a vacuum interrupter which includes contacts in accordance with the present invention.

The vacuum interrupter has a pair of metal endplates 11, 12 to which are bonded respectively in a vacuumtight manner a pair of tubular insulators 13, 14. Bonded to and trapped between the insulators 13, 14 is a flange 15 which forms part of and supports a cylindrical shield 16.

The fixed contact 17 is secured in a vacuumtight manner to the endplate 11 and is provided with an external terminal 18 for connection in an external circuit; the movable contact 19 slides in a bush 20 fixed to endplate 12, and is connected to an actuator (not shown) which moves it between the open position shown, and the closed position in which it abuts the fixed contact 17. The movable contact 19 is connected, for example by means of a flexible conducting braid 21, to a second terminal; moreover, a flexible bellows device 22 is provided, one end of which is sealed to the movable contact 19, and the other end of which is sealed to the endplate 12.

In the first embodiment of the invention, a portion, including the arcing face, of one of the cooperating contacts 17, 19, is formed of silver-silicon material, and a portion including the arcing face, of the other of the contacts is formed of silver-nickel material. It is immaterial whether the fixed contact 17 is formed of silver-silicon material and the movable contact 19 is formed of silver-nickel material or vice versa.

Each of the contacts 17, 19, is of cylindrical form, and they abut one another (when closed) at their cooperating, flat, circular end faces 23, 24; the arc normally runs between these flat end faces. A small radius is formed between the flat, circular end faces 23, 24 and the respective cylindrical faces to avoid a sharp edge.

The silver-silicon contact was made by vacuum melting pure silver and pure silicon together in a pure graphic crucible. The high vacuum was maintained by diffusion pumps with liquid nitrogen vapor traps, and 'clean' conditions were adhered to. The metals were heated by a radio frequency coil, using a molybdenum susceptor, for 30 minutes at 1,050° C. and were then cast into ingots. The preferred proportions are 4-6 percent silicon and 96-94 percent silver by weight.

The ingots so produced were machined by normal machining methods to the form of the contact.

The silver-nickel contact was made by compacting nickel powder of about 5 microns particle size in a hydraulic press at a pressure of 15 tons per square inch, using a steel die and plunger. The compact was then sintered at high vacuum for 20 minutes at 800° C. and the sintered compact was then infiltrated with pure silver at high vacuum in a graphite crucible for 10 minutes at 1,050° C. The infiltrated compact was machined to the form of the contact by normal machining methods. Analysis of a contact formed in this way showed that the operating face contained between 70 and 80 percent by weight of nickel. The preferred nickel content is between 65 and 85 percent by weight.

Operation of a high-vacuum interrupter having one silver-silicon contact and one silver-nickel contact made as described above showed that arcing between the cooperating faces of the contacts resulted in intermixing of the materials and the formation of nonductile films of nickel silicides on the cooperating faces. A large number of phases are believed to be formed, including  $\text{Ni}_2\text{Si}$ , and  $\text{Ni}_3\text{Si}_2$  and  $\text{NiSi}_2$ .

It was found that the contacts were mechanically strong and had high electrical and thermal conductivities, and that the

tendency of the contacts to weld together, or for surface grains or metallic filaments of the contacts to be drawn out as a result of partial welding of the contacts, was markedly reduced.

5 It will be understood that the formation of such filaments, or whiskers, may affect the contact life, and may also seriously reduce the voltage withstand of the contacts when in the open position.

10 Although the invention is not limited to the use of the contact materials described above, it will be appreciated that in determining the suitability of materials it is necessary to take into account not only the properties discussed above, but also other factors well known to those skilled in the art such as the current chopping characteristics.

15 In addition to the method described above, the silver-silicon contact may be formed by mixing silver powder and silicon powder (for example in the proportions 90 percent silver, 10 percent silicon by weight); when the powders are thoroughly 20 mixed, the resulting powder is compacted in a press at a pressure of 10 tons/sq. in., and the resulting 'compact' is sintered in vacuo at 790° C. for 45 minutes. This method overcomes certain difficulties which may occur with the vacuum melting and casting method described above, especially where an appreciable proportion, for example over 5 percent, of silicon is present.

25 In the second embodiment of the invention a portion, including the arcing face, of one of the cooperating contacts 17, 19 is formed of high-purity zone-refined copper, and a portion, including the arcing face, of the other of the contacts is formed of high-purity vacuum-outgassed titanium.

30 Operation of a high-vacuum interrupter having one high-purity zone-refined copper contact and one high-purity vacuum-outgassed titanium contact showed that arcing between the cooperating faces of the contacts resulted in the formation of nonductile films of copper-titanium compounds, and that there was a reduced tendency of the contacts to weld together.

I claim:

40 1. A vacuum circuit interrupter comprising an evacuated envelope and first and second contacts movable relatively to one another for contact engagement and disengagement within the envelope at cooperating contact regions, at said contact regions the first contact comprising nickel and the second contact comprising silicon; an arc struck between the contacts when separated during a circuit interruption causing the nickel and the silicon to mix with one another on the contact regions and to combine thereon to form surface films constituted by at least one nickel silicide, the material of the films forming a weld between the contacts when subsequently brought into engagement and being easily ruptured when the contacts are later separated.

45 2. A vacuum circuit interrupter comprising an evacuated envelope and first and second contacts movable relatively to one another for contact engagement and disengagement within the envelope at cooperating contact regions, at the said contact regions the first contact comprising silver-silicon and the second contact comprising silver-nickel.

50 3. A vacuum circuit interrupter according to claim 2, wherein at the respective contact region the first contact is a sintered particulate alloy of silver and silicon.

55 4. A vacuum circuit interrupter according to claim 3, wherein the sintered particulate alloy comprises approximately 90 percent silver by weight, the remainder silicon.

5. A vacuum circuit interrupter according to claim 2, wherein at the respective contact region the first contact is a cast alloy of pure silver and pure silicon.

60 6. A vacuum circuit interrupter according to claim 5, wherein the cast alloy comprises 94-96 percent silver by weight, the remainder silicon.

7. A vacuum circuit interrupter according to claim 2, wherein at the respective contact region the second contact is a sintered porous matrix of nickel having its pores infiltrated 75 with silver.

8. A vacuum circuit interrupter according to claim 7, wherein the sintered porous matrix of nickel having its pores infiltrated with silver comprises 65—85 percent nickel by weight, the remainder silver.

9. A vacuum circuit interrupter according to claim 8, wherein the sintered porous matrix of nickel having its pores infiltrated with silver comprises 70—80 percent nickel by weight, the remainder silver.